# EUROPEAN PATENT SPECIFICATION

(11) **EP 3 861 166 B1**
(45) Date of publication and mention of the grant of the patent: **14.01.2026**
(21) Application number: 19779046.2
(22) Date of filing: 04.10.2019
(51) Int. Cl.: D21F 11/00, D21H 27/10, D21G 1/00

(54) **KRAFT PAPER**
KRAFTPAPIER
PAPIER KRAFT

(30) Priority: 05.10.2018 EP 18198917
(43) Date of publication of application: 11.08.2021
(73) Proprietor: Billerud Aktiebolag (publ), 169 27 Solna (SE)
(72) Inventor: LINDSTRÖM, Ove, 952 91 Kalix (SE)
(74) Representative: Kransell & Wennborg KB
(86) International application number: PCT/EP2019/076953
(87) International publication number: WO 2020/070306

(56) References cited:
- EP-A1- 3 168 362
- EP-A2- 2 186 939
- DE-A1- 102010 029 580

## Description

### TECHNICAL FIELD

The present disclosure relates to the production of kraft papers as well as new kraft paper qualities.

### BACKGROUND

For many kraft paper applications, a smooth surface is desired, e.g. to improve printing quality. Calendering is frequently used for the purpose of obtaining such a smooth surface. Traditionally, calenders have been located at the end of the papermaking process (on-line). Paper has also been calendered separately (off-line) downstream the papermaking process.

The above-mentioned on-line and off-line calendering reduces the thickness of the paper. This generally considered a disadvantage for products that require a high bending stiffness since bending stiffness, as is well known, is strongly dependent on the thickness.

Extended soft nip calenders, such as belt calenders or shoe calenders, have been developed to limit the thickness reduction caused by calendering.

EP 3168362 B1 discloses i.a. a kraft paper having a density of 840 kg/m³, a strain at break in the machine direction (MD) of 2.2% and a bending resistance index in the MD of 234 Nm⁶/kg³, wherein one side of the kraft paper has a roughness of 470 ml/min.

### SUMMARY

The present inventor found that if a paper web is gently calendered in a moist state (i.e. before drying has been completed), surface properties of the resulting paper are significantly improved and the thickness is reduced but, unlike conventional calendering, the bending stiffness (measured as bending resistance) is not decreased. In many cases, the bending resistance is even increased in both directions of the paper.

The present disclosure enables the production of a new paper quality.

According to the invention, there is provided a single-layer kraft paper having:
- a density measured according to ISO 534:2011 of 720-850 kg/m³;
- a strain at break measured according to SS-ISO 1924-3:2011 in the machine direction (MD) of 1.0-2.9 %, such as 1.9-2.5 %; and
- a bending resistance index measured according to ISO 2493-1:2010 in the MD of 190-250 Nm⁶/kg³, such as 200-240 Nm⁶/kg³,
wherein at least one side of the kraft paper has a Bendtsen roughness measured according to ISO 8791-2 of 300-700 ml/min and wherein the kraft paper is formed from a paper pulp comprising at least 80 % by dry weight softwood pulp.

### DESCRIPTION

According to a first, non-claimed, aspect of the present disclosure, there is provided a method of producing a kraft paper having a strain at break in the machine direction (MD) of 1.0-8.9 %. In the present disclosure, the strain at break values are measured according to the standard SS-ISO 1924-3:2011

The density of the kraft paper is preferably 630-870 kg/m³. In embodiments of the first aspect, it is 690-850 kg/m³, such as 700- 830 kg/m³, such as 730-830 kg/m³. In the present disclosure, density is measured according to ISO 534:2011.

The grammage of the kraft paper may be 50-140 g/m². Preferably, it is 60-125 g/m².

In a particularly preferred embodiment, the grammage is 70-90 g/m², such as 75-85 g/m², when the strain at break in the MD is 1.0-2.9 % (see the third aspect discussed below). In the present disclosure, grammage is measured according to ISO 536:2012.

In another particularly preferred embodiment, the grammage is 95-130 g/m², such as 100-125 g/m², when the strain at break in the MD is 3.0-4.5 % (see the fourth aspect discussed below)
**The method** of the first aspect comprises a step of calendering a paper web at a dry content of 55-79 %, wherein the line load of the calendering step is 8-90 kN/m. A preferred dry content in the calendering step is 55-75 %. The line load is preferably 10-70 kN/m, such as 12-50 kN/m. In a particularly preferred embodiment, it is 15-40 kN/m. Benefits of line loads of ≤ 40 kN/m are shown in the examples section below.

This type of "wet" calendering, which uses a relatively low line load, surprisingly improves surface properties without decreasing the bending stiffness in the machine direction (MD). It may even improve the bending stiffness, in particular in the MD, even though it decreases the thickness of the paper. This is further discussed above in the summary section and shown below in the examples section.

The improved surface properties may be represented by relatively low Bendtsen roughness values. As an example, the Bendtsen roughness of at least one side of the kraft paper of the first aspect may be in the range of 300-700 ml/min. In the present disclosure, Bendtsen roughness is measured according to ISO 8791-2.

When the strain at break in a direction of the paper increases, the bending resistance the same direction typically decreases. Therefore, it may be preferred to avoid too high strain at break values when stiffness is a desired property. Accordingly, the strain at break in the MD of the kraft paper of the first aspect may be kept within the range of 1.0-6.0 %.

In embodiments of the first aspect wherein the strain at break in the machine direction (MD) of the kraft paper is 1.0-2.9 %, the bending resistance index in the MD of the kraft paper may be 190-250 Nm⁶/kg³ (see the third aspect discussed below).

In embodiments of the first aspect wherein the paper web is compacted in a Clupak unit, the strain at break values in the MD of the kraft paper are typically higher, i.e. 3.0-8.9 % and preferably 3.0-6.0 %. In such embodiments, the bending resistance index in the MD of the kraft paper may be 90-120 Nm⁶/kg³, such as 95-115 Nm⁶/kg³ (see the fourth aspect discussed below).

In the present disclosure, bending resistance is measured according to ISO 2493-1:2010. In this method, a bending angle of 15° and a test span length of 10 mm are used. To obtain the bending resistance index, the bending resistance is divided by the cube of the grammage.

The calender used for the calendering of the first aspect is preferably a soft nip calender, i.e. a calender in which a nip is formed between a roll with a hard surface, such as a metal surface, and a roll with a soft surface, such as a polymer-covered roll.

When a Clupak unit is used in the method of the first aspect, the paper web is preferably compacted in the Clupak unit before the step of calendering. As well known to the skilled person, a Clupak unit micro-crêpes the paper web (compacts the paper web in the machine direction) such that the strain at break values increases in the MD.

The calender for the calendering step of the first aspect is preferably arranged in a drying section of a paper machine. In such a drying section, the paper web is thus dried before and after the calendering step.

The kraft paper of the first aspect is preferably a single-layer kraft paper. A paper produced using two or more headboxes is not a "single-layer" paper according to the present disclosure. Nor is a laminate a "single-layer" paper according to the present disclosure.

Also for a porous sack paper, the combination of a relatively high stiffness and a relatively fine surface is of interest. As an example, high stiffness is often beneficial when the sack paper is converted to sacks and a finer surface improves the quality of a print on the sack paper. As a second, non-claimed, aspect of the present disclosure, there is thus provided a method of producing a sack paper. The sack paper of the second aspect is relatively porous in the sense that it has a Gurley value of less than 15 s. A typical lower limit for the Gurley value is 2 s or 3 s. The skilled person knows how to produce sack paper of such Gurley values (see e.g. WO 99/02772, which i.a. teaches to carry our HC refining, reduce the degree of LC refining (or even omit LC refining) and increase the dosing of strengthening agent). In the present disclosure, the Gurley value is measured according to ISO 5636-5:2013.

The improved surface properties may be represented by relatively low Bendtsen roughness values. As an example, the Bendtsen roughness of at least one side of the sack paper of the second aspect may be in the range of 300-700 ml/min.

The method of the second aspect comprises the steps of compacting a paper web in a Clupak unit and calendering the paper web at a dry content of 55-79 %, wherein the line load of the calendering step is 8-90 kN/m. A preferred dry content and preferred line loads are discussed above in connection with the first aspect.

The density of the sack paper is typically 670-800 kg/m³, such as 680- 750 kg/m³. The grammage of the sack paper may be 50-140 g/m². Preferably, the grammage is 60-120 g/m², such as 65-100g/m².

For sack papers, higher strain at break values are particularly preferred as they correspond to higher TEA values (and TEA is generally considered to be the value that best represents the relevant strength of the paper sack wall, which is supported by the correlation between TEA and drop test results). Accordingly, the strain at break in the MD of the sack paper may be 5.0-15.0 %. As well known to the skilled person, such strain at break values may be obtained if a Clupak unit is used in the production.

To provide strength, the sack paper of the second aspect is preferably a kraft paper.

As discussed above in connection with the first aspect, reduced stiffness is however often a side effect of increased strain at break values. Accordingly, a preferred sack paper produced according to the second aspect has a MD strain at break value in the range of 5.0-7.0 %, such as 5.0-6.5 %, and a bending resistance index in the MD of 86-108 Nm⁶/kg³.

The calender used for the calendering of the second aspect is preferably a soft nip calender (further discussed above in connection with the first aspect).

In the method of the second aspect, the paper web is preferably compacted in the Clupak unit before the step of calendering.

The calender for the calendering step of the second aspect is preferably arranged in a drying section of a paper machine. In such a drying section, the paper web is thus dried before and after the calendering step.

As understood by the skilled person, the methods of the first and the second aspect are carried out in a paper machine comprising a forming section (e.g. a wire section), a press section and a drying section. The paper web is thus formed in the forming section, dewatered in the press section and dried in the drying section to produce the kraft paper (first aspect) or porous sack paper (second aspect).

The present disclosure enables the production of a new kraft paper quality, which is particularly suited for packages for flour and sugar, especially the smaller packages of 0.5-2.5 kg found in grocery stores. This paper, which is provided as a third aspect of the present disclosure, is a single-layer kraft paper that has:
- a density of 720-850 kg/m³;
- a strain at break in the machine direction (MD) of 1.0-2.9 %, such as 1.9-2.5 %; and
- a bending resistance index in the MD of 190-250 Nm⁶/kg³, such as 200-240 Nm⁶/kg³,
wherein at least one side of the single-layer kraft paper has a Bendtsen roughness of 300-700 ml/min.

The density of the kraft paper is of the third aspect is preferably 730- 830 kg/m³, such as 750-830 kg/m³. The grammage of the kraft paper of the third aspect is preferably 50-140 g/m², such as 60-120 g/m², such as 65-100g/m², such as 70-90 g/m². In a particularly preferred embodiment, the grammage is 75-85 g/m².

The strain at break in the cross direction (CD) of the kraft paper of the third aspect may be 6.0-10.0 %, such as 7.0-9.0 %. Such a relatively high CD stretchability is beneficial as it results in high TEA values, which are beneficial in flour and sugar packages (to prevent package rupture).

The geometric tensile energy absorption (TEA) index of the kraft paper of the third aspect may for example be 1.9-2.2 J/g. In the present disclosure, the TEA values are measured according to the standard SS-ISO 1924-3:2011. To obtain the TEA index, the TEA value is divided by the grammage.

The geometric TEA index is calculated as the square root of the product of the TEA index in MD and CD:$geometric TEA index = √ \left(TEA index\left(MD\right)*TEA index\left(CD\right)\right) .$

The bending resistance index in the CD of the kraft paper of the third aspect may be 70-110 Nm⁶/kg³, such as 80-100 Nm⁶/kg³.

The Gurley value of the kraft paper of the third aspect is preferably 25-60 s, such as 25-45 s. Such Gurley values are beneficial during filling of the flour or sugar packages.

There is also provided a use of the kraft paper of the third aspect for forming a package for flour or sugar. Similarly, there is provided a method of forming a package for flour or sugar comprising the step of converting a paper of the third aspect into the package. The method may further comprise the step of filling the package with sugar or flour or another powdered food and optionally sealing the package after filling. This does not exclude other uses of the paper of the third aspect.

The present disclosure enables the production of another new kraft paper quality, which is particularly suited for sacks for flour and sugar, especially the larger sacks of 10-20 kg that are delivered e.g. to bakeries. This paper, which is provided as a fourth, non-claimed, aspect of the present disclosure, is a single-layer kraft paper that has:
- a density of 735-835 kg/m³;
- a strain at break in the machine direction (MD) of 3.0-4.5 %, such as 3.5-4.5 %; and
- a bending resistance index in the MD of 118-158 Nm⁶/kg³, such as 118-148 Nm⁶/kg³, such as 118-138 Nm⁶/kg³,
wherein at least one side of the kraft paper has a Bendtsen roughness measured according to ISO 8791-2 of 250-700 ml/min, such as 300-700 ml/min.

The density of the kraft paper of the fourth aspect is preferably 750- 830 kg/m³, such as 750-820 kg/m³.

The grammage of the kraft paper of the fourth aspect may be 50-140 g/m², such as 80-130 g/m². To provide enough strength for the above-mentioned sack for flour or sugar, the grammage is preferably 95-130gjm². In a particularly preferred embodiment, the grammage is 100-125 g/m².

The strain at break in the cross direction (CD) of the kraft paper is of the fourth aspect may be 6.0-10.0 %, such as 7.0-9.0 %. Such a relatively high CD stretchability is beneficial as it results in high TEA values, which are beneficial in flour and sugar sacks (to prevent sack rupture).

The geometric tensile energy absorption (TEA) index of the kraft paper of the fourth aspect may for example be 2.4-2.8 J/g.

The Gurley value of the kraft paper of the fourth aspect is preferably 18-60 s, such as 20-40 s.

There is also provided a non-claimed use of the kraft paper of the fourth aspect for forming a sack for flour or sugar. Similarly, there is provided a non-claimed method of forming a sack for flour or sugar comprising the step of converting a paper of the fourth aspect into the sack. The method may further comprise the step of filling the sack with sugar or flour or another powdered food and optionally sealing the sack after filling. This does not exclude other uses of the paper of the fourth aspect.

All papers of the present disclosure are preferably bleached, which typically means a brightness of at least 78 % or at least 80 % according to ISO 2470-1:2016. Preferably, a brightness of a bleached paper of the present disclosure is at least 81 %, such as 81-89 % (ISO 2470-1:2016).

To provide high tensile strength (which contributes to high TEA), the starting material used for preparing the pulp that is used for forming the papers of the present disclosure comprises softwood (which has long fibers and forms a strong paper). Accordingly, the papers of the present invention are formed from a paper pulp comprising at least 80 %, such as at least 90 %, softwood pulp. The percentages are based on the dry weight of the pulp.

Preferably, only virgin pulp is used for forming the papers of the present disclosure.

### EXAMPLES

### Example 1 (non-claimed)

Full-scale trials were carried out to produce white stretchable papers on a paper machine that is also used for producing sack paper. Both wet-calendered paper and non-calendered (reference) paper was produced.

The production is described below.

A bleached softwood sulphate pulp was provided. The pulp was subjected to high consistency (HC) refining (180 kWh per ton paper) at a consistency of about 39 % and low consistency (LC) refining (65 kWh per ton paper) at a consistency of about 4.3 %. Cationic starch (7 kg per ton paper), rosin size (2.4 kg per ton paper) and alum (3.5 kg per ton paper) were added to the pulp. In the headbox, the pH of the pulp/furnish was about 5.8 and the consistency of the pulp/furnish was about 0.3 %. A paper web was formed on a wire section. The dry content of the paper web leaving the wire section was about 19 %. The paper web was dewatered in a press section having two nips to obtain a dry content of about 38 %. The dewatered paper web was then dried in a subsequent drying section having ten dryer groups, including one Clupak unit, arranged in series. In this context, the Clupak unit was thus considered to be a "dryer group". The Clupak unit was arranged as dryer group seven, which means that the paper web was dried in the drying section both before and after being compacted in the Clupak unit.

When entering the Clupak unit, the moisture content of the paper web was 40 %. The hydraulic cylinder pressure exerted on the nip bar was set to 30 bar, resulting in a line load of 33 kN/m. The hydraulic cylinder pressure stretching the rubber belt was set to 31 bar, resulting in a belt tension of 7 kN/m. To reduce the friction between the paper web and the steel cylinder in the Clupak unit, a release liquid (1.5 % polyethylene glycol) was added in an amount of 250 litre/hour. The speed of the paper web in dryer group eight, which was the dryer group arranged directly downstream the Clupak unit, was 11 % lower than the speed of the paper web entering the Clupak unit.

A downstream portion of dryer group nine was rebuilt to comprise a soft calender nip (i.e. a nip between a roll having a hard (steel) surface and a roll having a soft (rubber) surface). The paper web was thus slightly dried between the Clupak unit and the soft calender nip, such that the web of the paper was subjected to calendering at a moisture content of 35 %. The line load was varied (see table 1). The temperature of the steel roll of the soft calender nip was about 100 °C. The reference paper was not subjected to calendering.

The properties of the papers produced in the trials are presented in table 1 below.

**Table 1. Paper properties of wet-calendered paper and non-calendered paper. The sample taken "After jumbo roll and winding" was obtained from the top (i.e. an outer layer) of a customer roll.**

| Trial | Wet-calendered paper | Wet-calendered paper | Wet-calendered paper | Wet-calendered paper | Non-calendered (reference) paper |
|---|---|---|---|---|---|
| Sample taken | After jumbo roll and winding | Top of jumbo roll | Top of jumbo roll | Top of jumbo roll | Top of jumbo roll |
| Wet calendering line load (kN/m) | 30 | 30 | 40 | 50 | 0 |
| Grammage (g/m²) | 150 | 150 | 150 | 150 | 150 |
| Thickness (µm) | 175 | 178 | 176 | 175 | 200 |
| Density (kg/m³) | 861 | 859 | 867 | 870 | 765 |
| Stretchability MD (%) | 14.8 | 14.7 | 14.3 | 15.0 | 14.6 |
| Stretchability CD (%) | 9.6 | 10.0 | 9.7 | 9.8 | 9.9 |
| TEA index MD/CD (J/g) | 6.8/3.0 | 6.7/3.2 | 6.3/3.2 | 6.6/3.2 | 6.6/3.2 |
| Burst index (mN/kg) | 5.0 | 5.0 | 5.3 | 5.2 | 4.8 |
| Bending resistance MD (mN) | 180 | 190 | 175 | 169 | 165 |
| Bending resistance CD (mN) | 194 | 191 | 193 | 155 | 169 |
| Bending resistance index MD (Nm⁶/kg³) | 53.3 | 56.3 | 51.9 | 50.1 | 48.9 |
| Bending resistance index CD (Nm⁶/kg³) | 57.5 | 56.6 | 57.2 | 45.9 | 50.1 |
| Gurley value (s) | 82 | 86 | 92 | 103 | 57 |
| Bendtsen roughness, SS* (ml/min) | 738 | 747 | 806 | 749 | 1451 |
| Bendtsen roughness, RS** (ml/min) | 1492 | 1793 | 1728 | 1688 | 3541 |

| | | | | | |
|---|---|---|---|---|---|
| * Steel side in calender, ** Rubber side in calender | | | | | |

Table 1 shows that the method of Example 1 falls outside the scope of the present invention due to high stretchability and high Gurley values. Table 1 still demonstrates, however, that wet-calendering significantly improves surface properties. In particular, the side of the paper contacting the (hard) steel roll in the wet calendering step obtained a fine surface (low Bendtsen roughness) independently of the line load. Surprisingly, it can thus be concluded that it was not necessary to use high line loads to obtain a significantly reduced Bendtsen roughness. More surprisingly, it was found that the wet calendering generally did not decrease the stiffness (measured as the bending resistance index) of the paper. Instead, the bending resistance index in the MD was increased for all line loads tested despite that the thickness was reduced by the wet calendering. The lower line loads (≤ 40 kN/m) even increased the bending resistance in both the MD and the CD.

Table 1 also illustrates that the winding of the paper to a jumbo roll and the subsequent winding to a customer roll improve the surface properties. The properties of the paper samples taken from the top of the jumbo roll are not a fair representation of the paper that is shipped to the customer. However, the effects seen by comparing paper samples taken from the same position are still valid.

### Example 2

Full-scale trials were carried out to produce white papers on a paper machine that is also used for producing sack paper. Two wet-calendered papers (trials 2 and 5), one final-calendered paper (trial 1) and two non-calendered papers (trials 3 and 4) were produced.

The production is described below.

### Example 2 - trials 1-3

A bleached softwood kraft pulp (100% virgin fibres) was provided. The pulp was subjected to high consistency (HC) refining (159 kWh per ton paper) at a consistency of about 35 % and low consistency (LC) refining (84 kWh per ton paper) at a consistency of about 4 %. Cationic starch (7.1 kg per ton paper), rosin size (2 kg per ton paper) and alum (2.9 kg per ton paper) were added to the pulp. In the headbox, the pH of the pulp/furnish was about 5 and the consistency of the pulp/furnish was about 0.25 %. A paper web was formed on a wire section. The dry content of the paper web leaving the wire section was about 18 %. The paper web was dewatered in a press section to obtain a dry content of about 42 %.

The dewatered paper web was then dried in a subsequent drying section having 8 dryer groups, including one Clupak unit, arranged in series. In this context, the Clupak unit was thus considered to be a "dryer group". The Clupak unit was arranged as dryer group 5, which means that the paper web was dried in the drying section both before and after the Clupak unit.

In trials 1-3, the Clupak unit was not operating and the paper web passed it without being compacted. In trials 4 and 5, the paper was however compacted in the Clupak unit (described below).

A soft nip calender was arranged between the Clupak unit and the following dryer group (the steel roll of the soft nip calender faced the wire side of the paper web). The temperature of the steel roll of the soft calender nip was about 50°C. In trial 2, the paper web was subjected to calendering in the soft nip calender at a dry content of about 65%. The pressure of the soft nip calender was set to 2.6 bar, corresponding to a line load of 15 kN/m. In trials 1 and 3, the soft nip calender was not operating and the paper web passed it without being calendered.

After the soft nip calender, the paper was further dried in dryer groups 6-8 to obtain a moisture content of 7.5 %.

A soft nip calender was arranged after the last dryer group (the steel roll faced the wire side of the paper web). The temperature of the steel roll of this soft calender nip was about 100 °C. In trial 1, the paper web was subjected to final calendering in this soft nip calender at a line load of 100 kN/m. In trials 2 and 3, the final soft nip calender was not operating and the paper web passed it without being calendered.

### Example 2 - trials 4 and 5

A bleached softwood kraft pulp (100% virgin fibres) was provided. The pulp was subjected to high consistency (HC) refining (284 kWh per ton paper) at a consistency of about 35 % and low consistency (LC) refining (93 kWh per ton paper) at a consistency of about 4 %. Cationic starch (8.6 kg per ton paper), rosin size (3.7 kg per ton paper) and alum (4.9 kg per ton paper) were added to the pulp. In the headbox, the pH of the pulp/furnish was about 5 and the consistency of the pulp/furnish was about 0.25 %. A paper web was formed on a wire section. The dry content of the paper web leaving the wire section was about 18 %. The paper web was dewatered in a press section to obtain a dry content of about 42 %.

The dewatered paper web was then dried in a subsequent drying section having 8 dryer groups, including one Clupak unit, arranged in series. In this context, the Clupak unit was thus considered to be a "dryer group". The Clupak unit was arranged as dryer group 5, which means that the paper web was dried in the drying section both before and after the Clupak unit.

In trials 4 and 5, the paper was compacted in the Clupak unit.

A soft nip calender was arranged between the Clupak unit and the following dryer group (the steel roll of the soft nip calender faced the wire side of the paper web). The temperature of the steel roll of the soft calender nip was about 50 °C. In trial 5, the paper web was subjected to calendering in the soft nip calender at a dry content of 65%. The pressure of the soft nip calender was set to 2.6 bar, corresponding to a line load of 15 kN/m. In trial 4, the soft nip calender was not operating and the paper web passed it without being calendered.

After the soft nip calender, the paper was further dried in dryer groups 6-8 to obtain a moisture content of 7.5%.

A soft nip calender was arranged after the last dryer group (the steel roll faced the wire side of the paper web). In trials 4 and 5, the final soft nip calender was however not operating and the paper web passed it without being calendered.

The properties of the papers produced in the trials 1-5 of Example 2 are presented in table 2 below.

**Table 2. "BR" means bending resistance. "BRI" means bending resistance index. "B. roug." means Bendtsen roughness. "TS" means top side. "WS" means wire side.**

| Trial | 1 | 2 (inventive) | 3 | 4 | 5 (non-claimed) |
|---|---|---|---|---|---|
| Clupak operating (yes/no) | no | no | no | yes | yes |
| Calendering | final | wet | no | no | wet |
| Grammage (g/m²) | 80.53 | 79.33 | 78.27 | 79.98 | 79.80 |
| Thickness (µm) | 93.62 | 102.07 | 112.85 | 109.88 | 101.51 |
| Density (kg/m³) | 860.18 | 777.21 | 693.58 | 727.88 | 786.13 |
| Stretchability MD (%) | 2.10 | 2.25 | 2.29 | 6.50 | 4.90 |
| Stretchability CD (%) | 7.38 | 7.40 | 10.90 | 9.45 | 7.58 |
| TEA index MD/CD (J/g) | 1.45/3.05 | 1.54/2.88 | 1.63/3.68 | 2.50/3.00 | 2.38/2.69 |
| TEA index geomet. (J/g) | 2.10 | 2.11 | 2.45 | 2.74 | 2.53 |
| Burst index (mN/kg) | 5.0 | 5.5 | 4.9 | 6.8 | 6.7 |
| BR MD (mN) | 85 | 111 | 102 | 44 | 53 |
| BR CD (mN) | 43 | 44 | 38 | 36 | 36 |
| **BRI** MD (Nm⁶/kg³) | 162.8 | 222.3 | 212.7 | 86.0 | 104.3 |
| BRICD (Nm⁶/kg³) | 57.5 | 56.6 | 57.2 | 45.9 | 50.1 |
| Gurley (s) | 52.69 | 39.16 | 49.38 | 23.75 | 25.64 |
| B. roug. TS (ml/min) | 264 | 554 | 1376 | 1226 | 473 |
| B. roug. WS (ml/min) | 203 | 483 | 1 007 | 706 | 401 |

Table 2 shows that wet-calendering significantly improves surface properties (compare trial 2 to trial 3 and trial 5 to trial 4). The line load of the "wet" calendering can be increased to e.g. 30 or 40 kN/m to further improve the Bendtsen roughness values, in particular those of trial 2. Further, table 2 confirms that that wet calendering generally does not decrease the stiffness (measured as the bending resistance index) of the paper despite a reduction of the thickness (compare trial 2 to trial 3 and trial 5 to trial 4). Instead, the bending resistance index in the MD was increased for both the Clupak-compacted and the non-compacted paper. For the non-compacted paper, the bending resistance index was increased also in the CD (compare trial 2 to trial 3).

By decreasing the compacting of the paper of trial 5 in the Clupak, an MD stretchability in the range of 3.0-4.5 % can be obtained. It is expected that such a decrease of the MD stretchability will increase the bending resistance index in the MD to a value in the range of 118-158 Nm⁶/kg³.

Based on the data in tables 1 and 2, it is expected that a wet-calendered paper will have significantly better surface properties than a final-calendered paper of the same bending resistance index. Consequently, the present disclosure i.a. facilitates production of paper with significantly improved surface properties without sacrificing any stiffness.

### Example 3

Full-scale trials were carried out to produce porous sack paper on a sack paper machine. Two wet-calendered sack papers (trials 2 and 3) and one non-calendered sack paper (trial 1) were produced.

A bleached softwood kraft pulp (100% virgin fibres) was provided. The pulp was subjected to high consistency (HC) refining and low consistency (LC) refining. Cationic starch, rosin size and alum were added to the pulp. In the headbox, the pH of the pulp/furnish was about 5.8 and the consistency of the pulp/furnish was about 0.25 %. A paper web was formed on a wire section. The dry content of the paper web leaving the wire section was about 18 %. The paper web was dewatered in a press section to obtain a dry content of about 42 %.

The dewatered paper web was then dried in a subsequent drying section having ten dryer groups, including one Clupak unit, arranged in series. In this context, the Clupak unit was thus considered to be a "dryer group". The Clupak unit was arranged as dryer group seven, which means that the paper web was dried in the drying section both before and after being compacted in the Clupak unit.

A downstream portion of dryer group nine was rebuilt to comprise a soft calender nip (i.e. a nip between a roll having a hard (steel) surface and a roll having a soft (rubber) surface). The paper web was thus slightly dried between the Clupak unit and the soft calender nip. The temperature of the steel roll of the soft calender nip was about 100 °C. In trials 2 and 3, the paper web was subjected to calendering in the soft nip calender at a dry content of about 70%-75%. In trial 2, the line load was 25 kN/m and in trial 3, it was 55 kN/m. In trial 1, the soft nip calender was not operating and the paper web passed it without being calendered.

After the soft nip calender, the paper was further dried to obtain a moisture content of 7.7%.

The properties of the papers produced in the trials 1-3 of Example 3 are presented in table 3 below.

**Table 2. "BR" means bending resistance. "BRI" means bending resistance index. "B. roug." means Bendtsen roughness. "TS" means top side (which faced the steel roll of the soft calender nip). "WS" means wire side (which faced the steel cylinder in the Clupak unit and the soft roll of the soft calender nip).**

| Trial | 1 | 2 (non-claimed) | 3 (non-claimed) |
|---|---|---|---|
| Calendering | no | wet (25 kN/m) | wet (55 kN/m) |
| Grammage (g/m²) | 82.24 | 81.06 | 80.44 |
| Thickness (µm) | 118.18 | 108.94 | 105.68 |
| Density (kg/m³) | 695.89 | 744.08 | 761.17 |
| Stretchability MD (%) | 3.99 | 3.88 | 4.41 |
| Stretchability CD (%) | 9.79 | 9.11 | 9.13 |
| TEA index MD/CD (J/g) | 1.82/3.10 | 1.93/2.81 | 2.09/3.06 |
| Burst index (mN/kg) | 4.2 | 4.3 | 4.3 |
| BR MD (mN) | 59 | 61 | 53 |
| BR CD (mN) | 38 | 37 | 38 |
| BRI MD | 106.7 | 114.5 | 101.8 |
| (Nm⁶/kg³) | | | |
| BRICD (Nm⁶/kg³) | 68.3 | 69.5 | 73.0 |
| Gurley (s) | 5.20 | 6.20 | 7.00 |
| B. roug. TS (ml/min) | 1246 | 655 | 677 |
| B. roug. WS (ml/min) | 717 | 564 | 547 |

Table 3 shows that wet-calendering significantly improved the surface properties, but that increasing the line load from 25 to 55 kN/m had no significant impact in this regard. Further, table 3 confirms that that wet calendering has no significant negative impact on the stiffness (measured as the bending resistance index) of the paper despite a reduction of the thickness. Some bending resistance index values were even increased by the wet calendering operation. It is further notable that wet calendering at 25 kN/m only increased the Gurley value by 1.0 s (when the line load was 55 kN/m, the increase was 1.8 s). The fact that the increase was not higher is of course advantageous when a paper that must be porous is produced.

The conclusions from Example 3 is that wet calendering is better than no calendering and that when wet calendering has been selected, 25 kN/m is a more preferred line load than 55 kN/m.

## Claims

1. A single-layer kraft paper having:
- a density measured according to ISO 534:2011 of 720-850 kg/m³;
- a strain at break measured according to SS-ISO 1924-3:2011 in the machine direction (MD) of 1.0-2.9 %; and
- a bending resistance index measured according to ISO 2493-1:2010 in the MD of 190-250 Nm⁶/kg³, such as 200-240 Nm⁶/kg³,
wherein at least one side of the kraft paper has a Bendtsen roughness measured according to ISO 8791-2 of 300-700 ml/min and wherein the kraft paper is formed from a paper pulp comprising at least 80 % by dry weight softwood pulp.

2. The kraft paper according to claim 1, wherein the density measured according to ISO 534:2011 is 730-830 kg/m³, such as 750-830 kg/m³.

3. The kraft paper according to any one of the preceding claims, wherein the grammage measured according to ISO 536:2012 is 50-140 g/m², such as 60-120 g/m², such as 65-100g/m², such as 70-90 g/m².

4. The kraft paper according to claim 3, wherein the grammage is 75-85 g/m².

5. The kraft paper according to any one of the preceding claims, wherein the strain at break measured according to SS-ISO 1924-3:2011 in the cross direction (CD) is 6.0-10.0 %, such as 7.0-9.0 %.

6. The kraft paper according to any one of the preceding claims, wherein the geometric tensile energy absorption (TEA) index measured according to the standard SS-ISO 1924-3:2011 is 1.9-2.2 J/g.

7. The kraft paper according to any one of the preceding claims, wherein the Gurley value measured according to ISO 5636-5:2013 is 25-60 s, such as 25-45 s.

8. The kraft paper according to any one of the preceding claims, which is formed from a paper pulp comprising at least 90 % by dry weight softwood pulp.

9. Use of the kraft paper according to any one of the preceding claims for forming a package for flour or sugar.

10. A method of forming a package for flour or sugar comprising the step of converting a paper according to any one of claims 1-8 into the package.

11. The method of claim 10, further comprising the step of filling the package with sugar or flour or another powdered food and optionally sealing the package after filling.

12. The method of claim 11, further comprising the step of sealing the package after filling.

## Patentansprüche

1. Einschichtiges Kraftpapier, aufweisend:
- eine Dichte von 720-850 kg/m³, gemessen nach ISO 534:2011;
- eine Bruchdehnung in Maschinenrichtung (MD) von 1,0-2,9 %, gemessen nach SS-ISO 1924-3:2011; und
- einen Biegefestigkeitsindex in MD von 190-250 Nm⁶/kg³, beispielsweise 200-240 Nm⁶/kg³, gemessen nach ISO 2493-1:2010
wobei mindestens eine Seite des Kraftpapiers eine Bendtsen-Rauhigkeit von 300-700 ml/min aufweist, gemessen nach ISO 8791-2, und wobei das Kraftpapier aus einem Papierstoff gebildet ist, der mindestens 80 Gew.-% Nadelholz-Zellstoff aufweist.

2. Kraftpapier nach Anspruch 1, wobei die nach ISO 534:2011 gemessene Dichte 730-830 kg/m³ beträgt, beispielsweise 750-830 kg/m³.

3. Kraftpapier nach einem der vorhergehenden Ansprüche, wobei das nach ISO 536:2012 gemessene Flächengewicht 50-140 g/m² beträgt, beispielsweise 60-120 g/m², beispielsweise 65-100 g/m², beispielsweise 70-90 g/m².

4. Kraftpapier nach Anspruch 3, wobei das Flächengewicht 75-85 g/m² beträgt.

5. Kraftpapier nach einem der vorhergehenden Ansprüche, wobei die nach SS-ISO 1924-3:2011 in Querrichtung (CD) gemessene Bruchdehnung 6,0-10,0 % beträgt, beispielsweise 7,0-9,0 %.

6. Kraftpapier nach einem der vorhergehenden Ansprüche, wobei der nach SS-ISO 1924-3:2011 gemessene geometrische Zugenergieabsorptions- (TEA) Index 1,9-2,2 J/g beträgt.

7. Kraftpapier nach einem der vorhergehenden Ansprüche, wobei der nach ISO 5636-5:2013 gemessene Gurley-Wert 25-60 s beträgt, beispielsweise 25-45 s.

8. Kraftpapier nach einem der vorhergehenden Ansprüche, das aus einem Papierstoff gebildet ist, der mindestens 90 Gew.-% Nadelholz-Zellstoff aufweist.

9. Verwendung von Kraftpapier nach einem der Ansprüche 5 bis 8 zur Bildung einer Verpackung für Mehl oder Zucker.

10. Verfahren zum Bilden einer Verpackung für Mehl oder Zucker, aufweisend den Schritt des Umformens eines Papiers nach einem der Ansprüche 1 bis 8 in die Verpackung.

11. Verfahren nach Anspruch 10, ferner aufweisend den Schritt des Befüllens der Verpackung mit Zucker oder Mehl oder einem anderen pulverförmigen Lebensmittel und optional des Verschließens der Verpackung nach dem Befüllen.

12. Verfahren nach Anspruch 11, ferner aufweisend den Schritt des Verschließens der Verpackung nach dem Befüllen.

## Revendications

1. Papier kraft monocouche présentant :
- une densité mesurée selon la norme ISO 534:2011 comprise entre 720 et 850 kg/m³ ;
- un indice d'allongement à la rupture mesuré selon la norme SS-ISO 1924-3:2011 dans le sens machine (MD) compris entre 1,0 et 2,9 % ; et
- un indice de résistance à la flexion mesuré selon la norme ISO 2493-1:2010 dans le sens machine (MD) compris entre 190 et 250 Nm⁶/kg³, tel que compris entre 200 et 240 Nm⁶/kg³,
dans lequel au moins un côté du papier kraft a une rugosité Bendtsen mesurée selon la norme ISO 8791-2 comprise entre 300 et 700 ml/min et dans lequel le papier kraft est formé à partir d'une pâte à papier comprenant au moins 80 % en poids sec de pâte de bois tendre.

2. Papier kraft selon la revendication 1, dans lequel la densité mesurée selon la norme ISO 534:2011 est comprise entre 730 et 830 kg/m³, telle que comprise entre 750 et 830 kg/m³.

3. Papier kraft selon l'une quelconque des revendications précédentes, dans lequel le grammage mesuré selon la norme ISO 536:2012 est compris entre 50 et 140 g/m², tel que compris entre 60 et 120 g/m², tel que compris entre 65 et 100 g/m², tel que compris entre 70 et 90 g/m².

4. Papier kraft selon la revendication 3, dans lequel le grammage est compris entre 75 et 85 g/m².

5. Papier kraft selon l'une quelconque des revendications précédentes, dans lequel l'allongement à la rupture mesuré selon la norme SS-ISO 1924-3:2011 dans le sens transversal (CD) est compris entre 6,0 et 10,0 %, tel que compris entre 7,0 et 9,0 %.

6. Papier kraft selon l'une quelconque des revendications précédentes, dans lequel l'indice d'absorption d'énergie géométrique à la traction (TEA) mesuré selon la norme SS-ISO 1924-3:2011 est compris entre 1,9 et 2,2 J/g.

7. Papier kraft selon l'une quelconque des revendications précédentes, dans lequel la valeur Gurley mesurée selon la norme ISO 5636-5: 2013 est comprise entre 25 et 60 s, telle que comprise entre 25 et 45 s.

8. Papier kraft selon l'une quelconque des revendications précédentes, qui est formé à partir d'une pâte à papier comprenant au moins 90 % en poids sec de pâte de bois tendre.

9. Utilisation du papier kraft selon l'une quelconque des revendications précédentes pour former un emballage pour de la farine ou du sucre.

10. Procédé de formation d'un emballage pour la farine ou le sucre, comprenant l'étape consistant à convertir un papier selon l'une quelconque des revendications 1 à 8 en emballage.

11. Procédé selon la revendication 10, comprenant en outre l'étape consistant à remplir l'emballage avec du sucre ou de la farine ou un autre aliment en poudre et, éventuellement, à sceller l'emballage après le remplissage.

12. Procédé selon la revendication 11, comprenant en outre l'étape consistant à sceller l'emballage après le remplissage.
